

July 20, 1926.

1,593,205

J. H. YOUNG

BUILDING MATERIAL

Filed Dec. 19, 1921

*Fig. 1.*



*Fig. 2.*



*Inventor:*  
James Howard Young  
*by* J. H. Churchill  
*Atty.*

## UNITED STATES PATENT OFFICE.

JAMES HOWARD YOUNG, OF PITTSBURGH, PENNSYLVANIA, ASSIGNOR TO H. H. ROBERTSON COMPANY, OF PITTSBURGH, PENNSYLVANIA, A CORPORATION OF PENNSYLVANIA.

## BUILDING MATERIAL.

Application filed December 19, 1921. Serial No. 523,359.

The present invention relates to an improved article of manufacture having an exterior metal surface, which is affixed to a foundation or underlying member by a 5 layer of asphalt or like bituminous material.

The present application is a continuation in part of my application filed March 27, 1920, Serial No. 369,294, in that it claims certain subject-matter disclosed but not 10 claimed in said application.

The invention has for its object to provide an article of the character described, which is highly resistant to the deleterious action of the weather, acid and alkali fumes, 15 and fire, and which can be produced at a minimum cost so as to be commercially available as a relatively inexpensive and durable material for building purposes.

The foundation or underlying member 20 may be of metallic or non-metallic material, either rigid or flexible, and in the present instance said foundation member is represented as a metal sheet, such as is now used in building constructions for roofing and 25 siding purposes, and to facilitate description, said foundation member will be hereinafter referred to as a metal sheet.

The metal sheet is provided with a layer 30 of asphalt or like bituminous material, by which the metal sheet is protected against corrosion and the action of acid and alkali fumes, and said asphaltic layer may be used alone or in conjunction with a sheet of 35 fibrous material such as asbestos felt or paper which is saturated with said bituminous material and affixed thereby to the metal sheet, as now commonly practiced in the manufacture of asphalt protected metal sheets and such as shown and described in 40 U. S. Patent No. 1,277,755 dated September 3, 1918. The asphalt or like bituminous layer is provided with an exterior surface or coating of metal, preferably lead, zinc, copper or like so-called non-corrodible 45 metals, which surface is composed of a layer of finely divided metal particles which are embedded in the asphaltic layer, and an additional layer of finely divided metal particles which are molecularly united with the 50 metal particles embedded in the asphaltic layer.

The finely divided particles of metal forming the layer which is embedded in the asphalt layer are projected into the asphalt

layer, and the finely divided particles forming the metallic layer which is molecularly united with the first mentioned metallic layer are projected against the embedded particles under sufficient pressure to weld or molecularly unite the metal particles of 55 both layers and thus provide the article to be protected with a metal surface or coating of substantially uniform thickness which conforms to the contour of the bituminous 60 covered article.

The metal coating or surface may be made of any desired thickness, as succeeding layers 65 of metal particles may be projected upon and molecularly united with the underlying 70 layer of metal particles.

The metal coating or surface may be made of a sufficient number of molecularly united 75 layers to provide a non-porous coating or surface upon the asphalt layer, but it is preferred to employ a relatively thin metal coating or surface which is more or less porous, as by so doing provision is made for the escape of the volatile ingredients in the asphalt and blistering of the metal coating 80 is thereby prevented.

These and other features of this invention 85 will be pointed out in the claims at the end of this specification.

Fig. 1 is a plan of a sufficient portion of 90 one form of protected metal sheet embodying the invention to enable it to be understood, and

Fig. 2, a section on an enlarged scale taken 95 on the line 2—2, Fig. 1.

Referring to the drawing, *a* represents the 100 article to be protected, which as above stated will be designated a metal sheet, which in the present instance is covered on all sides and edges with a layer *b* of asphalt or like bituminous material. The asphalt layer *b* is provided with a protective metal coating 105 composed of a plurality of layers of finely divided metal, such as lead, zinc, copper and the like, and in the present instance, two layers *c*, *d*, are herein represented. The metal layers *c*, *d* are composed of finely divided metal particles 10, 12, respectively, which are projected upon the asphalt coated metal sheet *a* with any suitable apparatus, as for instance, substantially that shown and 110 described in U. S. Patent No. 495,107 dated April 11, 1893.

The finely divided metal particles are

projected against the asphalt coated metal sheet *a* while the asphalt coating is in a more or less tacky or yielding condition and preferably soon after the asphalt coating 5 has been applied to the metal sheet, with the result that the metal particles 10, which strike against the asphalt layer *b* penetrate into and are embedded in the asphalt layer, and as they encounter a minimum resistance, they retain their original shape which, for sake of distinction, is represented in Fig. 2 as round or spherical, and thus form the underlying or embedded metal layer *c*. On the other hand, the metal particles 12 which 10 are projected against the layer *c* of embedded metal particles, strike the same with sufficient force to generate heat sufficient to cause the metal particles to cohere at their contacting points or surfaces and become 15 welded or molecularly united and form the metal layer *d*, which is thus molecularly united or welded to the underlying or embedded metal layer *c*. The metal particles 20 comprising the overlying or exterior layer *d*, are more or less distorted or changed from their original shape by impact against the particles of the underlying layer *c*, and this change or distortion is represented by 25 the irregular or other than round shape of 30 the particles comprising the exterior or surface layer, as represented in Fig. 2.

It is evident that by going over the asphalt covered metal sheet with the finely divided metal particles a sufficient number 35 of times or by going over the asphalt coated metal sheet slowly enough, a plurality of layers *d* may be built upon the embedded layer *c*, to provide the asphalt coated metal sheet with a non-porous metal coating composed of the underlying embedded layer *c* and a plurality of overlying or welded layers *d*, but it is preferred to provide the asphalt coated metal sheet *a* with a metal coating which is more or less porous for two purposes, to wit, to prevent blistering as above 40 described and to economize in the cost of the protected metal sheet, which result may be obtained with a single metal layer *d* welded to the embedded layer *c*. 45 The exterior metal surface or coating is firmly affixed to the asphalt coated metal sheet, and a highly efficient protected article is obtained, which is especially useful for building purposes, as the exterior metal surface or coating *c*, *d* efficiently protects the asphalt against deterioration and thereby prolongs the value of the latter for protecting the metal sheet *a* against corrosion, and also enables the finished article to be commercially used substantially as soon as produced, as it can be immediately packed, and shipped to the job, thereby avoiding the necessity of storing and drying and the expense attending the same, before the asphalt 55 covered metal article could be handled,

packed and shipped as is now required with asphalt coated metal articles now commonly prepared and known to me. Considerable difficulty has heretofore been experienced in the shipment of protected metal sheets of the character having a bituminous exterior surface or coating because of the fact that, in practice, these sheets are piled one upon the other and due to the weight of the steel, there is considerable pressure developed, 70 which causes the adjacent bituminous coatings to fuse together, which results in the sticking together of the separate sheets composing the pile. The separation of the individual sheets which are stuck in a pile usually results in damaging the protecting layers. It will be observed that the present metallic coating provides an anti-stick metallic coating which eliminates this difficulty. 80

Also the improved article is further available for building purposes, as a superior adhesion between the exterior metal coating or surface and the asphalt covered article is obtained, and the metal coating conforms to the contour of the asphalt coated article, is 85 non-inflammable and consequently highly advantageous as a protection against fire, and can be painted in any color, to obtain any article or pleasing design or color effect desired, as it has been found that the 90 metallic coating for the protected metal article is itself unaltered in color by the underlying bituminous layer and prevents discoloration of an ordinary paint film applied thereto. 95

Furthermore, the exterior metal coating when uncovered imparts to the asphalt covered article the naturally dull appearance of the metal which comprises the coating, and an exterior surface which is more or less rough or feathery in appearance, and when painted the relatively rough character of the metal coating affords an excellent surface for the adhesion of the paint. 100

#### Claims:-

1. A self supporting roofing or siding sheet comprising a steel sheet provided on one surface with a protecting layer of bituminous material, and a metallic coating covering the bituminous layer and which is formed as a part of the article, and also of a character whereby the protected sheet is provided with an external anti-stick metallic surface whose color or appearance is substantially uninfluenced by the bituminous material, and by virtue of which a plurality of the protected steel sheets may be piled for shipment superposed on one another and with bituminous surfaces in adjacent relation without liability of the sheets sticking together. 115

2. An improved article of manufacture composed of a foundation member having a layer of bituminous material thereon, and a metal coating for the bituminous layer 120

whose color or appearance is substantially uninfluenced by the bituminous layer, and which is formed as a part of the article, and comprising a layer of metal particles embedded in said bituminous layer, and a layer of metal particles molecularly united with the particles of the embedded layer.

3. An improved article of manufacture having a layer of bituminous material provided with a metal coating for the bituminous material, whose color or appearance is substantially uninfluenced by the bituminous material, and which is formed as a part of said article, and comprising a layer of metal particles embedded in said bituminous layer, and a layer of metal particles

molecularly united with the particles of the embedded layer.

4. An improved article of manufacture comprising a roofing material having a foundation member, a layer of bituminous material thereon, and a continuous and wholly metallic coating formed as a part of said article and itself composed of particles and imparting a relatively rough exterior metallic surface to the article, and providing the article with an exterior metallic surface whose color or appearance is substantially uninfluenced by the bituminous layer.

In testimony whereof, I have signed my name to this specification.

JAMES HOWARD YOUNG.